

Oct. 29, 1935.

L. D. MORTON

2,018,800

FIREPROOF THERMAL INSULATOR

Filed Aug. 29, 1931



Fig. 4



Fig. 5

Lawrence D. Morton INVENTOR.

BY

*H. S. Babcock*

ATTORNEY.

## UNITED STATES PATENT OFFICE

2,018,800

## FIREPROOF THERMAL INSULATOR

Lawrence D. Morton, Sandusky, Ohio, assignor to  
The Hinde & Dauch Paper Co., Sandusky, Ohio

Application August 29, 1931, Serial No. 560,119

12 Claims. (Cl. 154—45)

The invention to be hereinafter described relates to fire proof thermal insulators, and more particularly to what is known as the semi-rigid type of such insulators.

5 Any medium serving to prevent or retard the passage of heat may be regarded as a thermal insulator. A variety of materials in various combinations and forms have been used for this purpose.

10 Commercial heat insulators may be classified as of four types, namely: loose-fill insulation, flexible blanket type, rigid board type and semi-rigid board type. The ideal heat insulator, however, has been found to be an adequate space of still

15 air. Still air offers less heat conductance than any practical medium known.

That heat insulator which shall most nearly approach the ideal must be one in which still air is maintained with the least amount of material possible for practical use.

Heat insulation for buildings must comply with fire underwriters' restrictions in that it shall not be of a conflagratory nature.

20 It is also desirable that such insulation may be obtained in a form that may be readily and easily applied over any surface.

Considering the characteristics of the heat insulators on the market, one may observe that much improvement may yet be made.

25 The distinctive features which I have developed in my heat insulator are these: it shows, according to experts' tests, a higher heat insulating value, weight and volume considered, than any insulator other than still air, and that, although it is made wholly of paper, a highly combustible cellulosic material, it nevertheless resists combustion and cannot be made to conflagrate or burn of itself. It is fire proof.

30 A blow torch will slowly burn a hole in this insulating board, but cannot kindle it to self conflagration, for when the torch is removed the fire dies out quickly. This property is due partly to the construction of the board and to the fire-proofing cement used to bind its members together into a permanent structure.

35 The semi-rigid quality of this insulating board renders it particularly applicable to heat insulation of buildings. The board may be scored lengthwise or crosswise and bent to acute angles without breaking apart, and it does not appreciably warp or shrink.

40 The merits of my fire proof heat insulator, I have attained through a combination of materials and structure embodying certain principles

which I shall further set forth in the following specification, drawing and claims.

To produce an effective heat insulator, as defined in the earlier part of this application, I provide substantially parallel walls between 5 which air is constrained from circulating by cellular structure composed of as small a volume of inflammable cellulosic matter as is practical and the whole held together in a permanent structure with a fire-proofing cement.

10 Explicitly, the structure of my heat insulating board is as follows: a plurality of flat and fluted sheets of thin close-textured paper are alternately superimposed one upon another between flat side sheets and secured along all contacting 15 faces with a fireproofing cement. As will hereinafter appear, such a structure comprises, approximately a minimum quantity of solid material of low thermal conductivity (paper) and, approximately, a maximum quantity of a material of the highest practical thermal insulation capacity (still air) the combination providing greatest possible efficiency in thermal insulation. This same structure facilitates thorough permeation of the board with carbon dioxide (CO<sub>2</sub>) 20 throughout an appreciable area concentric with any point of enforced combustion, and automatic retaining of such gas over and enveloping the burned area, rendering the insulator self extinguishing and fire proof.

25 In order to illustrate the construction herein described, reference should be had to the accompanying drawing forming part of the present application. Throughout the several figures of the drawing like reference characters designate the 30 same parts in the different views.

In the drawing:

Fig. 1 is a fragmentary perspective view of the invention;

Fig. 2 is a like view of a single ply;

Fig. 3 is a cross section on line 3—3 of Fig. 1, looking in the direction of the arrows;

Fig. 4 is a fragmentary perspective view of a single ply with sheet partly separated; and,

Fig. 5 is a front or edge view of Fig. 4.

45

In the specimen taken for illustration, a five ply construction is shown, each ply comprising, a fluted sheet 1 and a plain sheet 2, the two being secured together by fireproof cement applied along the ridges of the flutes. Five such plies with 50 an additional outside plain sheet to completely utilize the last set of flutes, makes a five-ply board such as shown in Fig. 1. It will be understood that the cement is applied on all ridges—those on both sides of the fluted sheets. In this 55

way, each plain sheet, lying between two fluted sheets, as it does, is securely cemented to every ridge contacting its respective faces. In the assembly, the cement covered ridge-contacts with the plain sheets, are continuous from end to end. 5 The result is a great plurality of continuous parallel small-diameter tubes completely sealed against circulation from one to another. Only a very narrow strip of each ridge is cement coated—just enough to correspond to that contacted by the 10 adjacent plain sheet. When first applied, it may be considered as a narrow thin cap, such as indicated, considerably exaggerated, at 3 in Fig. 5. As the plain sheet contacts the ridge, the cap will be spread laterally, very slightly, having minimum 15 thickness or depth at the line of contact and increasing outwardly from each side of the contact, as indicated. This makes a complete seal throughout the length of every flute. Due, partly, to the fibrous nature of the material, lateral spread of 20 the cement, as the sheets are brought together, is not entirely uniform. The outer boundaries of spread are somewhat irregular, as indicated at 4 in Fig. 4. It will be understood that the cement penetrates considerably and is appreciably 25 absorbed by the sheets it connects, very slightly increasing their thickness along such lines of contact, the total increase for a five ply board of the kind illustrated being about .022 of an inch, along the lines of contact. This provides a 30 permanent structure of tubes in which all tubes are independent and in which every tube is completely isolated from every other tube and, furthermore, one in which there is no possible looseness or chance of air circulation between the sheets, 35 at any point or at any time.

On reference to Figs. 4 and 5, it will be seen that the total area covered by cement is a small fraction, only, of the total sheet area. All but that small fraction is entirely unprotected by cement and is of a readily inflammable nature. Cement is not indicated in Figs. 1 and 2 as such indication would lead only to confusion because of the size of the views.

The low combustibility of the board is due 45 partly to the multiplicity of fine parallel, evenly distributed, thread-like strips of fireproofing cement used and to the fact that the small diameter long conduits formed by the flutes serve during enforced combustion of the board to receive and 50 retain carbon dioxide gas in ample quantities to extinguish existing, and block further combustion of the board as soon as the applied flame is withdrawn. The high temperature of the blow torch will, obviously, greatly expand the gases 55 of combustion (mostly carbon dioxide and water vapor) at the point of combustion. This high expansion forces the gases into and to an appreciable distance within the tubes, overcoming the friction of the walls. So, for an appreciable distance 60 radially from the burned spot, the tubes will be packed with carbon dioxide, forming a thick, heavy, fire quenching blanket completely enveloping and overlying the burned area. This will remain even for a considerable time after the 65 blow torch has been removed. The wall friction, checking the inward flow of the gas, maintains the tubes filled continuously back to and including their smoldering ends. This assures the effective, operative, smothering or enveloping position of 70 the gas blanket until it slowly dissipates, which is more than amply long enough to effect thorough and complete fire extinguishing.

Only within small limits can increases in the size of the flutes be made without impairing the

character of the board as a heat insulator and as a fire resistor. Increasing the size of the flues decreases wall friction or resistance to air circulation and diminishes ability to hold and retain carbon dioxide gas in a sufficient quantity, also the quantity of fireproofing cement would be proportionately insufficient to be effective. Evidently there is a means that must be met between an excess of cellulosic matter and an excess of total free air within the tubes or cells in a given 10 area and thickness of the board.

In the manufacture of corrugated paper and boxes made therefrom, silicate of soda is the most generally used cement. Silicate of soda or its equivalent, as an adhesive, is more effective than 15 cements which would be softened by water vapor. Because it is not affected by water vapor, it continues, as a skeleton-work, to hold the carbonized or charred paper intact to form a fire-proof shield between any flame and the unburned 20 paper underneath. But, other cements which would be softened by the water vapor would fail, the charred parts would fall away, and the unburned paper beneath would be exposed to the flame and burn. It would not be fireproof.

In the construction of my insulation I prefer to use a 25 lb. machine-glazed kraft paper of about .003 inch thickness. The fluted sheets have fifty-two flutes to the foot and are 3/32" thick measured from peak to valley, or, in the direction of the thickness of the fireproof insulator. In a five ply board of this insulation one-half inch thick the solid cellulosic stock thickness is approximately .040", leaving a still air space .460". In this preferred structure the total paper or 30 cellulosic solids will be found to be approximately, 7.70% of the entire volume. While this is cited as a preferred construction, I have obtained highly satisfactory results from a considerable range of other dimensions and proportions of paper, including 8, 9 and 10 plies per inch, of sheets of kraft paper ranging in thickness from .0025" to .004", and having from 36 to 52 corrugations to the foot. With fewer than 8 plies to the inch of thickness and 42 corrugations to the lineal foot, 40 from paper 16" wide, so that the flutes will be 16" long, the structure is not dependably fire proof when a blow torch is applied midway of the length of the corrugations. The increase in cross section of the tube, in proportion to the length, 45 appears to so reduce wall friction, that the carbon dioxide generated, expanded by the heat of the blow torch, apparently, flows too far into the tubes to act as an extinguisher at the charred ends. But, if the length of this same tube or 50 corrugation is increased sufficiently, as by making it from sheets 30" wide, for instance, the insulator becomes fire proof. Thus, 8 ply sheets of .003" and .004" paper with 36 corrugations to the foot are fire proof when made from paper 60 30" wide, giving flutes about 13" long from a burned center. Applying the same tests to an insulator of the preferred construction, specimens 16", 12" and 9" square were used. A blow torch burned a hole through the center of each, 65 leaving tubes substantially 6", 4" and 3" long, from the charred edges. It is not practical to apply a hot flame such as that of a blow torch to a sheet less than 9" x 9", as the spread of flame would practically envelope the whole surface of such a smaller sheet. They were all thoroughly fire proof. So, available data indicates that minimum length of tube is determined by the ratio between the peak-to-valley diameter and the length. That ratio must be such that 70 75

the wall friction of the tube will so retard the flow of carbon dioxide, when heated, as to hold it within the near ends of the tubes. Increase in length of tubes, apparently, permits increase 5 in peak-to-valley diameter. While there may be a minimum length for a given diameter of tube, there is, seemingly, no maximum, other than that imposed by manufacturing facilities.

As previously stated, there is, evidently, a mean

10 that must be met between an excess of matter and an excess of free air. Or, there is an approximate allowable proportion of total cellulosic solids relatively to total air. I have found that ten plies to the inch with 52 corrugations to the foot, 15 eight plies to the inch with 42 corrugations to the foot, and eight plies to the inch with thirty-six (36) corrugations to the foot, all gave fire proof insulators when made from machine glazed kraft paper .0025", .003" or .004" sheets. The 20 volume percentage of cellulosic solids in the above will be found to be, approximately, 10% in the densest, not appreciably over. When the volume of cellulosic solids is appreciably in excess of 10%, due to the use of more than 52 corrugations to the foot, or more than ten plies to the inch, or paper more than .004" in thickness, the insulator is no longer dependably fireproof. There then seems to be too great a percentage 25 of cellulosic solids. So, in constructing this fire- 30 proof insulator from paper, the total paper incorporated, apparently, should not appreciably exceed 10% of the total volume. Sheets thinner than .0025" are impractical of manufacture at the present time for this construction but are 35 thoroughly acceptable, otherwise and may be used when suitable facilities have been developed.

Kraft paper has been mentioned as the preferred type because it is easily obtained at a

40 moderate price in practically any locality, may be readily had in any desired widths (for tube lengths) and thicknesses, and because it has the desired closeness of texture and is well adapted to the corrugating process. Any other applicable papers may, obviously, be used.

45 The fireproof characteristics of this paper thermal insulator (100% highly inflammable cellulose) and air, are the result of:—

1st. So proportioning the flutes or tubes that, under enforced combustion they will frictionally 50 hold a smothering or fire quenching blanket of carbon dioxide over and about the burned area.

2nd. A multiplicity of fine thread-like parallel and closely spaced strips of fireproof cement which, as the insulator is burned, because the 55 cement is not softened by water vapor, maintains its skeleton or lattice-work and holds the carbonized paper in place as a fire shield between any flame and the unburned paper.

3rd. So proportioning the total still air and 60 its distribution relatively to the total cellulosic content and its distribution, as to provide less that the minimum cellulosic material necessary to support combustion, in such an assembly.

For insulation against heat where fire hazard is 65 not a question the size of flutes may be increased even to double the size, with ends closed; higher insulation values are obtained than with any other heat insulator known, weight and volume considered.

70 Maintaining the same quality of kraft paper as used in the half inch board and increasing the size of flutes, a five ply board one inch thick may be made having the same weight or less. The total still air space in such a board will be .960" 75 as the total stock thickness is still only .040".

While a five ply board has been illustrated and described, it will be understood that other numbers of plies may be used. Likewise, flutes of other shapes may be used, as, triangular, rectangular, elliptical, etc. The paper mentioned is 25 lb. machine-glazed kraft of about .003" thickness. Such designation is illustrative of a preferred paper but a number of other papers are thoroughly practicable though varying somewhat in the characteristics given. While applicant has, to a certain extent, as a means of illustration, specified certain materials and constructions, it is to be clearly understood that he is not in any degree limited to such illustrative disclosures. Many changes may be made, within 10 the scope of the appended claims, in the materials and constructions herein disclosed, without in any degree departing from the field of the invention, and it is meant to include all such within this application, wherein only a single preferred 15 form has been illustrated.

Having thus described my invention, what I claim and desire to protect by Letters Patent is:

1. A fireproof thermal insulator consisting of a plurality of paper tubes parallelly bound together in a permanent structure by thread-like narrow strips of fireproof cement along their lines of contact and completely sealing each from communication with the others, the volume of cellulosic solids bearing such a relation to the total 25 volume of air and cellulosic solids as to render the insulator incapable of sustaining combustion.

2. A fireproof thermal insulator consisting of a plurality of paper tubes parallelly bound together in a permanent structure by thread-like 35 narrow strips of fireproof cement along their lines of contact and completely sealing each from communication with the others, the cross sectional dimensions of said tubes bearing such relation to their lengths that said tubes, under enforced 40 combustion, retain carbon dioxide sufficiently to effect extinguishment.

3. A fire proof thermal insulator comprising a plurality of alternately disposed plane and corrugated sheets of paper of a thickness of the order of approximately .0025" to approximately 45 .004", fire proof cement securing said sheets permanently together and disposed in skeleton form comprising a plurality of spaced parallel thread-like strips between and connecting the sheets, 50 said insulator having the plane sheets spaced from .1" to .125" apart, approximately, both inclusive, each corrugated sheet having, approximately, from 36 to 52, both inclusive, corrugations per foot.

4. A fire proof thermal insulator comprising a plurality of alternately disposed planed and corrugated sheets of paper of a thickness of the order of approximately .0025" to approximately 60 .004", said insulator having the plane sheets 65 spaced from .1" to .125" apart, approximately, both inclusive, fire proof cement securing said sheets permanently together and disposed in skeleton form comprising a plurality of spaced parallel thread-like strips between and connecting the sheets, the total cellulosic solids of said insulator not appreciably exceeding 10% by volume of the entire insulator.

5. A fire proof thermal insulator comprising a plurality of alternately disposed plane and corrugated sheets of paper of a thickness of the order of approximately .0025" to approximately 70 .004", said insulator comprising a plurality of plies of said sheets, fire proof cement securing said sheets permanently together, each corrugated 75

gated sheet having approximately from 36 to 52, both inclusive, corrugations per foot, the total cellulosic solids of said insulator not appreciably exceeding 10% by volume of the entire insulator.

6. A fire proof thermal insulator comprising a plurality of alternately disposed plane and corrugated sheets of paper of a thickness of the order of approximately .0025" to approximately .004", said insulator having the plane sheets spaced from .1" to .125" apart, approximately, both inclusive, fire proof cement securing said sheets permanently together, along the lines of contact between the sheets and corrugations, each corrugated sheet having, approximately, from 36 to 52, both inclusive, corrugations per foot, the total cellulosic solids of said insulator not appreciably exceeding 10% by volume of the entire insulator.

7. A fire proof thermal insulator comprising a plurality of alternately disposed plane and corrugated sheets of paper of a thickness of the order of approximately .003", said insulator having the plane sheets spaced apart .1", approximately and each corrugated sheet having approximately 52 corrugations per foot, and fire proof cement permanently connecting said sheets along the lines of contact between said corrugations and said sheets.

8. A fire proof thermal insulator comprising alternately disposed plane and corrugated sheets of paper permanently secured in the formation of a plurality of parallel adjoining small diameter air containing tubes, a multiplicity of thread-like, closely spaced parallel strips of fire proof cement connecting said tubes and providing a skeleton work retaining frame, the cellulosic solids of said paper being uniformly distributed through said insulator and being between 5% approximately and 10% approximately of the total volume of said insulator.

9. A fire proof thermal insulator comprising a plurality of alternately disposed plane and cor-

rugated sheets of paper of a thickness from approximately .0025" to approximately .004", said insulator having the plane sheets spaced from .1" to .125" apart, approximately, both inclusive, each corrugated sheet having approximately from 36 to 52, both inclusive, corrugations per foot, the total cellulosic solids of said insulator ranging between 5% approximately and 10% approximately of the total volume of said insulator, and fire proof cement permanently securing said sheets together along the lines of contact between said sheets and said corrugations.

10. A fire proof thermal insulator comprising a body of cellulosic material having a plurality of closely arranged permanent separate air containing tubes extending therethrough, the volume of cellulosic solids bearing such a relation to the total volume of air and cellulosic solids as to render the insulator incapable of sustaining combustion.

11. A fire proof thermal insulator comprising a body of cellulosic material having a plurality of closely arranged separate permanent air containing tubes extending therethrough, the cross sectional dimensions of said tubes bearing such a relation to their lengths that the insulator, under enforced combustion, will retain within said tubes carbon dioxide sufficiently to effectively extinguish combustion.

12. A fire proof thermal insulator comprising a body of cellulosic material having a plurality of closely arranged separate permanent air containing tubes extending therethrough, the volume of cellulosic solids bearing such relation to the total volume of cellulosic solids and air as to render the insulator incapable of sustaining combustion, and the cross sectional dimensions of the said tubes bearing such relation to their lengths that said tubes, under enforced combustion, retain carbon dioxide sufficiently to effect extinction.

LAWRENCE D. MORTON.